

Oct. 18, 1938.

J. C. HOSTETTER ET AL

2,133,768

INSULATOR

Filed Sept. 7, 1937



INVENTOR.  
JOHN C. HOSTETTER  
AND JESSE T. LITTLETON  
BY *Dorsey, Cole & Farmer*  
ATTORNEYS.

## UNITED STATES PATENT OFFICE

2,133,768

## INSULATOR

John C. Hostetter, West Hartford, Conn., and  
 Jesse T. Littleton, Corning, N. Y., assignors to  
 Corning Glass Works, Corning, N. Y., a corpora-  
 tion of New York

Application September 7, 1937, Serial No. 162,774

6 Claims. (Cl. 173—28)

This invention relates to insulators and par-  
 ticularly to those which are used in the open  
 and hence are exposed to varying weather con-  
 ditions.

5 In a prior Patent No. 2,118,795, issued May 24,  
 1938, to Jesse T. Littleton, there is described an  
 insulator, a portion of which is coated with tin  
 iridizing whereby an extremely thin layer of tin  
 compound having an appreciable electrical con-  
 ductivity is formed on its surface. Such a coating  
 10 eliminates the electrical brush discharge  
 known to the art as corona by preventing the  
 building up of a potential gradient between the  
 line wire and the surface of the insulator. The  
 15 potential gradient, which normally is present be-  
 tween any conductor of high potential and a  
 dielectric in contact therewith, is in this case  
 spread out and dispersed over the slightly con-  
 ducting tin iridized coating. It is further shown  
 20 in the above mentioned application that other  
 iridized coatings, such as those produced by iri-  
 dizing with silicon tetrachloride and salts of  
 tungsten and molybdenum which under proper  
 25 conditions likewise produce conducting coatings,  
 have a similar effect.

Insulators so treated are known as "no static"  
 insulators and are very desirable for power trans-  
 mission at high voltages, because the absence of  
 30 corona therein not only prevents leakage of power  
 but completely eliminates the "static" or radio  
 interference which has been a source of annoy-  
 ance in radio reception in the vicinity of power  
 lines and which was long sought to be overcome.

We have found that "no static" insulators, such  
 35 as those that are tin iridized, are subject to a  
 certain amount of deterioration in service in that  
 exposure to the weather and attendant electro-  
 lytic action causes a change in the iridized film,  
 which results in a gradual loss of its conductivity.  
 40 It is the object of this invention to prevent  
 loss of efficiency of conducting iridized coatings  
 on insulators.

We have now discovered that the weathering  
 45 of conducting iridized coatings on insulators may  
 be prevented by applying over such a coating an-  
 other iridized coating which has an extremely  
 high resistance particularly at relatively low volt-  
 ages and is hereinafter called a non-conducting  
 50 iridized coating. Although we believe that any  
 non-conducting iridized coating will have a pro-  
 tective effect as indicated by experiments made  
 with various non-conducting coatings produced  
 55 by iridizing with chlorides of iron, titanium, alu-  
 minum and silicon, we prefer to use iron iridizing

or titanium iridizing since these are relatively  
 easy to apply.

The invention therefore consists in the article  
 and the method of preparing it to be more fully  
 described in the following specification, claimed  
 in the appended claims and illustrated in the  
 accompanying drawing which shows an insulator  
 5 partly in section having an exaggerated tin iri-  
 dized zone which is covered over with iron iridizing,  
 also greatly exaggerated, in accordance with 10  
 our invention.

In practicing our invention it is preferable to  
 apply the coatings to the insulator as it is taken  
 from the mold at which time its temperature is  
 about 600° C. to 750° C., but on account of un-  
 15 even cooling in some types of insulators it is de-  
 sirable first to place the insulator in a reheat-  
 ing kiln held at about 650° C. in order that the  
 parts to be coated may be brought to proper tem-  
 perature. The above named temperatures are 20  
 effective for insulators made of low expansion  
 borosilicate glass, such as the glass B<sub>2</sub> of the  
 Sullivan and Taylor Patent No. 1,304,623, but  
 softer glasses will require relatively lower tem-  
 25 peratures as may be determined by trial.

The insulator is coated or "iridized" while hot,  
 either by spraying it with a solution of metal salt  
 or by exposing it to the fumes of the salt. For  
 example, a tin iridized coat is first applied by  
 spraying or atomizing on the part to be coated, 30  
 a water solution of stannous chloride containing  
 enough hydrochloric acid to prevent hydrolysis  
 or the vapor stannic chloride may be directed  
 against the insulator by blowing dry air through  
 35 liquid anhydrous stannic chloride in a suitable  
 container such as an Erlenmeyer flask provided  
 with a delivery tube. This salt is readily vapor-  
 40ized without the use of heat and the amount of  
 fumes is controlled merely by regulating the cur-  
 rent of air. Best results are obtained by intro-  
 ducing some moist air into the vapor jet as it  
 strikes the heated insulator surface. An ex-  
 45 tremely thin iridescent layer of oxide having a  
 low electrical resistance, approximately .001 ohm  
 per centimeter cube, is formed on the surface of  
 the glass and permanently incorporated there-  
 with. Various other salts of tin will produce the  
 same result.

Obviously only a portion of the insulator is  
 to be so coated with such a conducting coating 50  
 and this is accomplished by placing the hot insu-  
 lator on a rotating table and protecting the por-  
 tion which is not to be iridized with an asbestos  
 mask. The pinhole of the insulator may be iri-  
 55 zed by means of an additional nozzle or jet 55

placed in the center of the rotating table. An exposure to the spray or vapor for about five to fifteen seconds will suffice to produce the desired result.

5 After the tin iridized coat has been applied as above described, and before the insulator cools to any great extent, an iron iridized coating is immediately applied thereover. This may be accomplished by atomizing a water solution of 10 ferric chloride or by heating the solid salt in a closed container provided with a delivery tube. The spray or vapor is directed against the parts to be coated as before for about five to fifteen seconds. In this case it is desirable to use a different mask of such size and shape as will permit the iron iridized coating to extend beyond the limits of the tin iridized coat and preferably to extend to the edge of the insulator skirt as shown 15 in the drawing. If desired, the iron iridized coating may cover the entire insulator. This insures that the tin iridized coat will be completely covered and the entire upper surface of the insulator which is most exposed to the direct action of the weather will be covered with a highly 20 resistant protective coating.

25 In lieu of iron iridizing, titanium iridizing may be applied by using the vapor of titanium tetrachloride in a similar manner or other non-conducting iridized coatings disclosed in the above 30 mentioned prior patent may be used. For best results, however, the iron or titanium iridizing is preferred.

35 Analytical investigation has shown that these iridized coatings, both conducting and non-conducting, as described above, are composed of an oxide of the metal whose salt is employed in the iridizing process.

40 After the electrically conducting iridized coating and overlying non-conducting iridized coating have been applied, the insulator, if desired, may be annealed in the usual manner. The insulator could be annealed and cooled after the application of the tin iridized coat to be followed by reheating, application of the iron iridized coat 45 and subsequent annealing, but this procedure would obviously be uneconomical.

50 "No static" insulators, which have been treated in the above described manner with an overlying non-conducting iridized coating, will resist weathering effects better than those to which only a conducting iridized coating has been applied. Contrary to expectations, the application of a

non-conducting coating over the conducting coating does not hinder the corona-preventing effect of the conducting coating and, although the reason for this may not be thoroughly understood, it is believed that due to the thinness of the non-conducting coating the charging current from the line and tie wires builds up practically the same potentials over the conducting coating beneath as would exist were the non-conducting coating not present. In the case of some coatings, such 5 as the iron oxide coating, it has been found that the outer or insulating coat becomes conducting under the high voltage gradient of the line-to-pin potential so that the conducting under coat has practically the same potential and potential distribution as it would were it not covered, and hence the corona formation is prevented in the 10 normal manner. Yet this insulating coat is a perfect insulator to the low voltages causing the electrolytic destruction of the tin oxide coat. It 15 is believed that the protective non-conducting coating should not be excessively thick at the point where it contacts the line and the tie wires. When such coatings are applied too thickly they 20 lose their iridescent appearance. The proper 25 thickness will not be exceeded if the above recited instructions are observed.

We claim:

1. An insulator provided with an electrically 30 conducting iridized zone and a non-conducting iridized coating on the conducting iridized zone.
2. An insulator having an iridized conducting metallic oxide surface and an iridized non-conducting metallic oxide coating on the conducting surface.
3. An insulator provided with a tin iridized zone 35 and an iron iridized coating on the tin iridized zone.
4. An insulator provided with a tin iridized zone and a titanium iridized coating on the tin 40 iridized zone.
5. An insulator having an iridized surface of tin oxide and an iridized coating of iron oxide overlying and extending beyond the limits of the tin oxide surface.
6. An insulator having an iridized surface of tin oxide and an iridized coating of titanium oxide overlying and extending beyond the limits of the tin oxide surface.

50 JOHN C. HOSTETTER.  
JESSE T. LITTLETON.